

252-149

+ thickening agent

## United States Patent Office

3,041,285

Patented June 26, 1962

1

3,041,285  
COMPOSITION FOR CLEANING AND POLISHING  
ALUMINUM AND ALUMINUM ALLOYSKenneth Walter Newman, Van Nuys, Calif., assignor,  
by mesne assignments, to Purex Corporation, Ltd., a  
corporation of CaliforniaNo Drawing. Filed May 27, 1955, Ser. No. 511,779  
7 Claims. (Cl. 252—149)This invention relates to chemical compositions for 10  
the cleaning and polishing of aluminum and aluminum  
alloys.Principally, the object of the invention is to provide  
a chemical cleaner which will remove oxide, tarnish and  
other discoloring materials or soil from the surfaces of 15  
aluminum and aluminum alloys, without attacking the  
underlying pure aluminum or aluminum alloy surfaces.It is therefore a further and very important object of  
the invention to provide a chemical brightening or polishing  
agent for aluminum and aluminum alloys which will 20  
not attack the metal and therefore will not weaken the  
metal surfaces or promote danger of structural failure.A still further object is to provide a polisher or cleaner  
of the indicated nature which is especially adapted to  
the polishing of aircraft surfaces which are formed from  
aluminum and aluminum alloys. Such a composition 25  
must be in all respects safe, not in any way harmful to  
personnel who apply it, and not in any way corrosive to  
the base aluminum or aluminum alloy metal, even after  
water or other solvent employed is evaporated and even  
after the lapse of a considerable period of time, such 30  
as several weeks, wherein corrosive action, as between  
faying or contacting surfaces, might develop.Other objects of the invention, as well as the various  
features of novelty therein, will become apparent to those  
skilled in the art upon reference to the following specification  
wherein certain preferred embodiments are disclosed.Compositions of this invention include essentially  
thiourea and a relatively large proportion of a particular  
non-oxidizing, non-corrosive organic acid capable of  
yielding a pH below 3. The particular acid is glycolic  
acid, and the proportion of this acid is at least equal to  
that of the thiourea (by weight) and preferably consider- 40  
ably more, such as one and one-half times the thiourea,  
or twice, or even up to three or four or five times the  
thiourea. In aqueous solutions employing around 10 to  
20 times as much water as the acid, a pH between 2.0  
and 2.8 is yielded without being corrosive to aluminum 45  
or aluminum alloy surfaces. Such proportions of acid  
and thiourea are readily soluble in water, the solution  
is generally free from objectionable odor, and the solution  
also is relatively non-toxic to personnel employing the  
materials. Since thiourea is soluble in water to the ex- 50  
tent of only 9% to 10% by weight, and since a consider-  
able concentration of the acid is required, the high  
water solubility of this acid, at least to the extent of being  
soluble in an equal weight of water, is important. This  
solubility is additionally important when it is considered 55  
that a thickening agent is employed in the solution in  
order that the polish may be sprayed upon the metal or  
mopped upon the metal and be allowed to remain, without  
running off, for a considerable period of time, such  
as 15 minutes to 30 minutes or longer, before the cleaner 60  
is washed off or otherwise appropriately removed from  
the surface being cleaned.While metal cleaning solutions containing thiourea and  
acids have been known heretofore, none have been  
satisfactory for thorough cleaning of aluminum and alumi- 65  
num alloy surfaces, such as aircraft surfaces, particularly  
because of being highly corrosive to such surfaces.

2

In practice one part of thiourea is commonly employed  
with one and one-half to two or three parts by weight  
of glycolic acid, and these are used in about ten parts  
by weight of water to yield the required solution. Ordin- 5  
arily, the solution has added thereto a thickener in quantity  
to produce the desired consistency above described.  
Such a thickener might comprise about one-fourth part  
of methyl cellulose, or ethyl cellulose, or gum tragacanth,  
or hydroxyethyl carboxymethyl cellulose, or agar agar, or  
other similar thickener which will dissolve in the solu- 10  
tion and will subsequently wash off readily. As one use-  
ful example, about two parts by weight of glycolic acid  
is used with one part by weight of thiourea and these are  
dissolved in about ten parts by weight of water (sufficient  
to dissolve the thiourea), such solution yielding a pH 15  
around 2.2 to 2.5. One-fourth part by weight of methyl  
cellulose is added to yield a thickened solution which  
may be applied as such by spraying, brushing, or other-  
wise as desired.20 In a particular preferred instance I have employed the  
following composition (by weight):

|                  | Percent |
|------------------|---------|
| Glycolic acid    | 11      |
| Thiourea         | 6       |
| Water            | 81.7    |
| Methyl cellulose | 1.3     |

Another example of a desirable composition is the fol- 30  
lowing (by weight):

|                  | Percent |
|------------------|---------|
| Glycolic acid    | 7.5     |
| Thiourea         | 5.0     |
| Water            | 86.0    |
| Methyl cellulose | 1.5     |

35 In addition to the above particular examples, the pro-  
portions of thiourea, acid and water may be varied con-  
siderably, so long as there is adequate water to dissolve  
the thiourea. The thickener may be omitted when de-  
sired, and its proportion also may vary. Possible varia- 40  
tions in the composition are generally indicated by the  
following tables:

## Approximate Parts and Percentages

45

TABLE I

|           | Parts | Per- | Parts | Per- | Parts | Per- | Parts | Per- |
|-----------|-------|------|-------|------|-------|------|-------|------|
| Acid      | 1     | 8    | 1     | 8    | 2     | 15   | 3     | 20   |
| Thiourea  | 1     | 7    | 1     | 8    | 1     | 7    | 1     | 7    |
| Water     | 10    | 85   | 10    | 82   | 10    | 75   | 10    | 71.5 |
| Thickener |       |      | 1/4   | 2    | 1/2   | 3    | 10    | 1.5  |

TABLE II

55

|           | Parts | Per- | Parts | Per- | Parts | Per- | Parts | Per- |
|-----------|-------|------|-------|------|-------|------|-------|------|
| Acid      | 1     | 6    | 2     | 11   | 4     | 20   | 4     | 25   |
| Thiourea  | 1     | 6    | 1     | 5.5  | 1     | 5    | 1     | 6    |
| Water     | 15    | 85   | 15    | 83.5 | 15    | 75   | 10    | 65   |
| Thickener | 1/2   | 3    |       |      |       |      | 2/3   | 4    |

TABLE III

65

|           | Parts | Per- | Parts | Per- | Parts | Per- | Parts | Per- |
|-----------|-------|------|-------|------|-------|------|-------|------|
| Acid      | 1     | 5    | 2     | 10   | 3     | 13   | 4.3   | 16   |
| Thiourea  | 1     | 5    | 1     | 5    | 1     | 5    | 1     | 4    |
| Water     | 20    | 90   | 20    | 83   | 20    | 80   | 20    | 77   |
| Thickener |       |      | 3/2   | 2    | 2/3   | 2    | .7    | 3    |

While the above tables, showing approximate parts and percentages, indicate as little as 5% of glycolic acid with not more than an equal amount of thiourea, and a percentage of glycolic acid as high as 25% of the composition (4 to 5 times the thiourea), it is generally preferable to employ appreciably, but not greatly, more glycolic acid than thiourea, such as approximately twice as much as in the preferred example first listed above, or around one and one-half times as much as in the second example. As to the thickener, while about 1.5% is usual, more or less, or none at all, as indicated, is acceptable under varying conditions.

The possible over-all percentage ranges for the constituents, as represented by the examples and tables above, are thus as follows (by weight):

Glycolic acid, about 5% to 25%  
 Thiourea, about 4% to 8%  
 Water, about 65% to 90%  
 Thickener, 0% to 4%

While a limit of about 25% of glycolic acid has been indicated, it nevertheless would be possible sometimes to employ up to about 40% glycolic acid. In such a case, the water content would be about 55% to dissolve satisfactorily 5% of thiourea, this composition thus employing about nine parts of glycolic acid, one part of thiourea, and twelve parts of water.

The indicated acid proportions ordinarily yield pH values between 2.2 and 2.5, pH 2.0 to 2.8, that is less than about pH 3, being necessary to effect adequate cleaning to yield the required brightened metal surface.

From the standpoint of appropriate materials to clean aluminum and aluminum alloys, it is to be recognized that aluminum is an amphoteric metal and that its action is quite different from that of other metals. Thus, it is said in the work of Jenny and Lewis, entitled "Anodic Oxidation of Aluminum and Its Alloys," published by Chemical Publishing Co., Inc., New York, N.Y., in 1940, pages 50 and 51, that:

"In its behavior toward acids, aluminum differs greatly from other metals. . . . It is not the degree of dissociation of an acid, but the affinity of the aluminum for the anion which is the determining factor in the solution process."

As a consequence it will be appreciated that the acid above disclosed as providing for the proper cleaning of aluminum and aluminum alloys, without corrosion of the base metals, is an acid whose anion does not have corrosive affinity for aluminum and its alloys, which is non-oxidizing, and yet which, in the required concentrations, provides the indicated 2.0 pH to 2.8 pH to dissolve the various oxides, sulphides and other staining and soiling constituents which must be removed to yield the bright or polished surface which is required and which, as produced by the present invention, glistens and gleams as though the surface had been hand polished and hand buffed. Such a condition is accomplished merely by mopping or spraying onto the metal surface a composition as above described, which necessarily contains glycolic acid as the acid constituent, allowing it to remain on the metal surface for a period of from about fifteen minutes to about thirty minutes, scrubbing the surface preferably with a stiff brush or similar rubbing instrument, and then rinsing the surface thoroughly with water, as from a hose, whereby to leave the surface clean and polished. When the composition is to be mopped or wiped on the surface to be cleaned, it preferably contains an indicated thickener, though not necessarily so. When the solution is to be sprayed on the surface, the thickener might be omitted, though not necessarily so because the thickener restricts run-off and also evaporation of the solvent.

As to the thiourea, it is possible to substitute simple alkyl derivatives thereof such as methyl or ethyl thiourea

and such are intended to be included by the term "thiourea" as used herein.

In addition to the indicated glycolic acid and thiourea, it may sometimes be desirable to include an appropriate wetting agent as is well understood, such as the various well known sulfonic acids and sulfonates prepared from fatty alcohols, fatty acids, fatty acid esters, and so on. Corrosion inhibitors also may be used, as well understood, when desired to protect other parts such as cadmium-plated steel rivets, bolts and other corrodible parts.

From the standpoint of an acid acceptable for the present purpose, I have found that glycolic acid is the only acid which is completely non-corrosive to aluminum and aluminum alloy surfaces, as above described, which will at the same time remove oxides, tarnish, other soil, staining, light corrosion as distinguished from heavy corrosion, and the like from aluminum and its alloys, without attacking the metal itself, which is non-oxidizing, and which has the required pH of about 2.0 to 2.8 in all concentrations of about 5% to 25% in the water solution.

The product in the various forms described may be packaged dry, the acid and thiourea appearing as crystals, the thickener, such as methyl cellulose, also appearing in dry form if used. Where the product is packaged dry, the required proportions of water will, of course, be added subsequently, such as at the time of use, in accordance with instructions which could appear on the package. Otherwise, the product may be packaged in solution form ready for use.

30 I claim as my invention:

1. A method for polishing aluminum and aluminum alloy surfaces which comprises the steps of: applying to such a surface a coating of a solution consisting essentially of one part thiourea and one to about five parts of glycolic acid in water providing a pH value between about pH 2 and pH 3; working such solution upon the surface to remove oxides and tarnishing constituents; and rinsing the treated surface with water.

2. A method as in claim 1 wherein the water of the cleaning solution amounts to about ten to twenty parts.

3. A method as in claim 1 wherein said solution remains in contact with said surface from about 15 minutes to 30 minutes to effect a thorough brightening thereof.

4. A method as in claim 1 wherein said solution contains a dissolved thickener retarding evaporation and run-off of the solution during the contact time.

5. A method as in claim 1 wherein the glycolic acid is present in the proportion of about three parts to one part of thiourea.

6. A liquid composition for polishing aluminum and aluminum alloy surfaces consisting essentially of: 1 part of thiourea; from 1 part to about 5 parts of glycolic acid, and from about 10 to 20 parts of water, said composition having a pH of between about 2 and 2.8.

7. The composition of claim 6 including a minor proportion of a thickening agent dissolved therein, wherein said composition has an increased viscosity and ability to be retained on the surfaces treated.

60 References Cited in the file of this patent

UNITED STATES PATENTS

|              |                                |                 |
|--------------|--------------------------------|-----------------|
| 1,608,622    | Schmidt et al. <i>252-149</i>  | Nov. 30, 1926   |
| 1,736,118    | Gravel -----                   | " Nov. 19, 1929 |
| 2,049,517    | Saukaitis -----                | " Aug. 4, 1936  |
| 65 2,186,579 | Dubpurnell et al. <i>134-3</i> | Jan. 9, 1940    |
| 2,270,712    | Wood <i>252-142</i>            | Jan. 20, 1942   |
| 2,318,559    | Percival -----                 | May 4, 1943     |
| 2,383,800    | Johnson <i>146</i>             | Aug. 28, 1945   |
| 2,511,988    | Myers <i>134-3</i>             | June 20, 1950   |
| 70 2,558,167 | Beghin et al. <i>252-136</i>   | June 26, 1951   |
| 2,586,331    | Hill <i>4 149</i>              | Feb. 19, 1952   |
| 2,593,259    | Brissey et al. <i>136</i>      | Apr. 15, 1952   |
| 2,607,722    | Kremel <i>142</i>              | Aug. 19, 1952   |

## UNITED STATES PATENTS

2,628,199 Lowenheim ~~252-142~~ Feb. 10, 1953  
2,672,449 Snell et al. ~~" 100~~ Mar. 16, 1954

## FOREIGN PATENTS

913,121 Germany ~~252-146~~ June 8, 1954  
1,038,238 France ~~" 142~~ May 6, 1953  
161,565 Australia ~~" "~~ Mar. 1, 1955

## OTHER REFERENCES

Corrosion Handbook by Uhlig, page 910, pub. by John Wiley, N.Y. (1948).  
5 Methocel, pages 2 and 17, pub. by Dow Chem. Co., Midland, Mich. (1949).